

1

2,878,119

## PROCESS FOR BLEACHING AND SIZING PAPER PULP

Charles R. Cutterson, Richmond, Va., and Richard S. Bell and Henry W. Ellerson, Jr., Roanoke Rapids, N. C., assignors to The Albermarle Paper Manufacturing Company, Richmond, Va., a corporation of Virginia

No Drawing. Application March 2, 1956  
Serial No. 568,962

12 Claims. (Cl. 92—21)

This invention relates to a new and improved process for bleaching sulfate paper pulp.

It has been the practice hitherto to bleach the paper pulp and then to wash it thoroughly to remove chlorinated lignins, oxidized color bodies, soluble salts, such as calcium salts produced by calcium hypochlorite bleaching, and other impurities prior to sizing of the paper furnish. Such separate preliminary bleach and wash operations have been the rule whether the bleaching is multi-stage to produce substantially fully bleached paper or single-stage to produce semi-bleached paper and require the installation and maintainance of expensive chlorination and wash equipment, additional manpower and considerably increased processing time. Where a semi-bleached pulp is suitable for the particular use, the added costs of separate bleaching and washing treatments is often prohibitive.

The object of this invention is to provide a process whereby sizing of sulfate paper pulp can be carried out either during the bleaching procedure or subsequent to bleaching but in the presence of the bleaching reaction by-products in such manner that separate bleaching equipment is rendered unnecessary.

Another object is to provide a process whereby bleaching and sizing of sulfate paper pulp can be performed in a single unitary operation.

Still another object is to eliminate washing of the bleached pulp as a separate operational procedure.

Other objects include the manufacture of semi-bleached kraft paper having excellent size and strength properties and good color at greatly reduced cost.

Broadly speaking, our process comprises admixing the sulfate pulp with hypochlorite bleach, such as calcium, sodium or potassium hypochlorite, allowing sufficient time for the bleaching oxidation and chlorination action of the hypochlorite to become effective, and then adding alum both to release the chlorine remaining in the residual hypochlorite and to set the rosin size. Rosin size is added at any time prior to addition of the alum or can be introduced subsequent to alum addition. Washing of the bleached pulp as a separate operation, whether the rosin is added in the presence of the hypochlorite or subsequent to alum addition, can be dispensed with since we have found that the aqueous dilution of the pulp which is required for sheet formation on the paper making machine can serve as an adequate wash mechanism if certain precautions are observed as will subsequently be described. Although, as aforementioned, other hypochlorites can be employed with equally satisfactory results, we prefer, in general, to employ calcium hypochlorite because of its low cost and ease of handling.

The amount of hypochlorite added to the sulfate pulp is determined largely by the bleach demand of the pulp, the degree of brightness desired and the amount of time which can be allowed for action of the bleach in terms of available equipment and economical processing. In general, we prefer to employ the hypochlorite in an amount which provides sufficient available chlorine to satisfy up

2

to about 70% of the bleach demand of the pulp since the pulp reacts with the bleach in such proportions quite rapidly, generally within a period of about  $\frac{1}{2}$  to 2 hours, and these amounts generally produce a semi-bleached

5 paper of good brightness for most purposes. It will be understood, however, that larger proportions of the hypochlorite as, for example, up to the total bleach demand, may be used but, because of the slowness of reaction after bleachability of the pulp has been reduced by about 60 to 10 70%, either considerably longer periods of time must be allowed for more complete bleaching action or substantial waste of unreacted bleach will be incurred.

Bleach requirement or bleachability of the pulp can be determined by any of the well known standard methods, 15 as, for example, by determination of the permanganate number or the number of milliliters of N/10 permanganate consumed by 1 gram of oven-dry pulp. The permanganate number can be converted into approximately equivalent chlorine in terms of hypochlorite for bleaching by use of the proper factor for the particular type of pulp.

20 The hypochlorite can be added to the pulp, if desired, in a separate mixing chest and the pulp then passed into the beater for the addition of the rosin size and alum. However, from the point of view of economic equipment utilization, we prefer to conduct the bleaching operation in the beater.

25 The hypochlorite can be introduced into the beater concurrently with the sulfate paper pulp or after the beater has been filled. Reaction of the hypochlorite with the lignins and other color-forming bodies in the pulp proceeds quite rapidly until an amount of hypochlorite providing available chlorine equivalent to about 60 to 70% of the bleach demand is consumed in both oxidation and chlorination reactions. If more hypochlorite is present, 30 reaction will generally continue much more slowly beyond this point.

35 The normal alkalinity of the sulfate pulp (generally in the neighborhood of about pH 9) provides substantially optimum conditions for the action of the hypochlorite, 40 both from the point of view of speed of reaction and minimizing degradation of the pulp. As reaction with the hypochlorite continues pH decreases, generally to about pH 7 or 8, due to formation of HCl and other acidic products.

45 The rosin size can be introduced into the paper furnish in the beater at any point prior to addition of the alum. It can be added before the hypochlorite, concurrently with the hypochlorite or subsequent to the addition of the hypochlorite. The rosin is entirely compatible with the hypochlorite in the pulp mixture. In some cases as, for example, where the paper pulp is passed in a continuous process through Jordan refiners, the rosin size can be added to the pulp in the refiners subsequent to the addition of the alum in the beater. In such case 50 the standard paper making practices employed where rosin is added after the alum should be followed. The rosin size should desirably be introduced in diluted form as, for example, about 1% solids concentration, to prevent loss of sizing uniformity because of rapid precipitation by the alum present. Since the bleached pulp is not 55 washed, the hypochlorite bleaching by-products remain in the pulp during sizing. However, their presence does not adversely affect sizing.

60 Any suitable rosin size can be employed, including 65 substantially completely saponified rosin in the form of sodium resinate, partially saponified rosin containing from small to substantial amounts of free rosin and free rosin size emulsions, such as Bewoid size. It will be understood that the term rosin as employed in the specification and claims encompasses the various types of rosin size, as 70 aforementioned. The rosin size furthermore can be employed in conjunction with such other sizing components

as wax emulsions and the like depending on the specific properties required in the paper.

It has generally been the consensus of opinion hitherto that the presence of calcium salts adversely affects the rosin sizing operation. It would appear, therefore, that the calcium salts, such as calcium sulfate formed upon addition of alum, which are a by-product of calcium hypochlorite bleaching, would exert a deleterious action on the rosin sizing. We have found, however, that sizing is actually improved when it is carried out in conjunction with the hypochlorite bleaching. In other words, with a given pulp, type and amount of size, improved sizing results, as for example, in terms of water resistance, are obtained when the hypochlorite bleach is applied during the sizing operation. This is an unexpected phenomenon, which, while we cannot at present satisfactorily explain it, is an important advantage of our process.

The amount of rosin size employed is that normally used in the paper making art for the particular type of pulp and desired finished paper characteristics.

Other materials which are ordinarily incorporated into the paper stock in the beater can be introduced as well as the rosin size, such as dyestuffs and fillers, so long as they are not chemically affected by the hypochlorite. The dyestuffs employed, for example, should be of the acid-fast type.

The action of the hypochlorite on the pulp is allowed to continue in the beater for a suitable length of time. The particular reaction period is determined by a number of factors such as the amount of hypochlorite employed, the temperature and concentration of the pulp, degree of brightness desired in the finished paper, practical considerations of permissible processing time and the like.

The alum which is then added to the beater serves a dual purpose. It eliminates the residual hypochlorite remaining in the pulp by reacting with it to release free chlorine which acts on the pulp to produce additional bleaching action, and it provides for precipitation or setting the rosin size whether the latter is introduced before or after. The amount of alum required to remove the residual hypochlorite over and above that normally employed to precipitate the size is generally quite small. We have found that the addition of alum in an amount sufficient to decrease pH of the pulp mix to about 6.0 or 6.5 is generally adequate both for satisfactory rosin fixing and hypochlorite elimination, though more may be added.

Concentration of the pulp can be at any workable level which can satisfactorily be handled by the available equipment. In most cases, the beater is geared to handle pulp concentrations of about 3 to 5 percent. Bleaching of the pulp according to our process is very satisfactory at these concentrations, particularly with regard to uniformity.

The treated pulp, after leaving the beater, can be subjected to ordinary paper-making routine. It can, for example, be dumped into a stuff or beater chest for routine storage and then pumped through refiners, where as aforescribed, rosin size can be introduced if sizing has not been performed in the beater during the hypochlorite treatment, thence to another stuff or machine chest and on to the paper making machine. If the stock is not subjected to refiner treatment, it can be passed directly from the beater or beater chest to the paper making machine.

One advantage of the standard practice of temporarily storing the beater contents in a beater chest prior to sheet formation on the paper making machine stems from the fact that this storage time gives such chlorine as has been released from the residual hypochlorite by the alum opportunity to act on and be absorbed by the pulp for further bleaching action.

When the bleached and sized pulp reaches the paper-making machine it is subjected to routine dilution in the head box for sheet formation on the wire screen. In routine paper making practice the pulp is diluted to a

consistency of about 0.2 to 0.5% although concentration may be as low as 0.1% and as high as 1% depending on the particular type of paper being made and the characteristics of the particular pulp such as type and length of the fibers and the like.

We have found that the water which is added to dilute the paper making stock prior to sheet formation and then drained off the paper machine wire provides adequate washing of the bleached pulp and removes a sufficient amount of the bleaching by-products and impurities to prevent any substantial color reversion. This method possesses the important advantage of eliminating a separate washing procedure along with the expensive equipment and additional processing time which this would require.

Fresh water can be employed for dilution of the paper making stock, if desired, for somewhat more thorough washing. However, the process can be more economically practiced by recirculating the white water effluent for stock dilution so long as care is exercised to avoid the use of water which has become substantially saturated with the bleach impurities since this will reduce the washing effect to the point where substantial color reversion will occur. This can be avoided by addition of some fresh water to the recirculated white water effluent as required.

The semi-bleached papers formed by our process are of excellent quality with regard to strength, size properties and brightness. The ordinary brown color of unbleached 30 kraft papers is reduced generally to a bright canary yellow. They are highly satisfactory for use in specialty wrapping papers, such as butcher paper, manila envelopes and folders, fiber cartons and the like.

### 35

#### Example I

800 lbs. of air dry sulfate pulp in the form of slush was furnished to a beater and reduced to a consistency of 4%. While the pulp was being introduced into the beater, a bleaching solution of calcium hypochlorite containing approximately 30 gms./liter of chlorine was also run in. The total quantity of bleach was equivalent to 4% chlorine based on the air dry fiber. Maleic fortified rosin size was then added to the beater contents in an amount corresponding to 1% by weight of the air dry fiber. 0.5% emulsified wax size by weight of the air dry fiber was then introduced. Beater action was continued for about 1 hour, after which alum was added in amount sufficient to precipitate the rosin and wax sizes and to acidify the entire beater contents to approximately pH 6.0.

The bleached and sized fiber was passed into a beater chest and then on to a Fourdrinier paper machine where it was diluted to a consistency of about 0.5% prior to sheet formation. Water drained from the sheet on the paper wire was recirculated to the head box for stock dilution.

Paper was made having a basis weight of 40 lbs. per ream of 500 sheets, size 24 in. by 36 in. Tests were made in accordance with ASTM designation D-779-54 to determine the degree of sizing. Results of 38 to 40 seconds were obtained, indicating a high degree of water resistance. The color of the paper was changed from brown to a pleasing canary yellow and brightness was improved by about 10 points, namely from Hunter 34 to 44. The permanganate number of the pulp was reduced from 26 to 17.

#### Example II

The same procedure was followed as in Example I except that the amount of calcium hypochlorite added was increased to the equivalent of 8% chlorine based on air dry fiber and the pulp was retained in the beater for 90 minutes.

The degree of sizing of the paper was about the same as in Example I. Brightness was improved by about 17

points, namely from Hunter 34 to 51 and permanganate number of the pulp was reduced from 26 to 12.

Although this invention has been described with reference to illustrative embodiments thereof, it will be apparent to those skilled in the art that it may be embodied in other forms but within the scope of the appended claims.

We claim:

1. A process for bleaching and sizing sulfate paper pulp which comprises admixing an aqueous slurry of the pulp with hypochlorite bleach, permitting the hypochlorite to react with the pulp for at least  $\frac{1}{2}$  hour and then adding alum in an amount sufficient to react with residual hypochlorite and to precipitate the rosin size, introducing rosin size into the pulp at any time prior to dilution of the pulp for sheet formation, whereby sizing of the paper pulp is accomplished in the presence of said hypochlorite bleach or its reaction products, then diluting said pulp with water to the consistency requisite for paper sheet formation, the maximum concentration of the pulp being about 1%, forming paper sheets with said diluted pulp and removing the water after said sheet formation, said dilution water serving as the only wash for said treated pulp.

2. The process of claim 1 in which the pulp concentration when treated with the hypochlorite is about 3 to 5%.

3. The process of claim 1 in which the hypochlorite is calcium hypochlorite.

4. The process of claim 2 in which the pulp concentration when treated with the hypochlorite is about 3 to 5%.

5. The process of claim 2 in which the calcium hypochlorite is added in an amount comprising up to the equivalent of about 70% of the bleach demand of the pulp.

6. The process of claim 5 in which the pulp concentration when treated with the hypochlorite is about 3 to 5%.

7. A process for bleaching and sizing sulfate paper pulp which comprises admixing an aqueous slurry of the pulp with hypochlorite bleach and rosin size, permitting the hypochlorite to react with the pulp for at least  $\frac{1}{2}$  hour and then adding alum in an amount sufficient to react with residual hypochlorite and to precipitate the rosin size, the rosin size being introduced into the pulp at any time prior to addition of the alum, whereby sizing of the paper pulp is accomplished in the presence of said hypochlorite bleach or its reaction products, then diluting said pulp with water to the consistency requisite for paper sheet formation, the maximum concentration of the pulp being about 1%, forming paper sheets with said diluted pulp and removing the water after said sheet formation, said dilution water serving as the only wash for said treated pulp.

8. The process of claim 7 in which the pulp concentration when treated with the hypochlorite is about 3 to 5%.

9. The process of claim 7 in which the hypochlorite is calcium hypochlorite.

10. The process of claim 9 in which the pulp concentration when treated with the hypochlorite is about 3 to 5%.

11. The process of claim 9 in which the calcium hypochlorite is added in an amount comprising up to the equivalent of about 70% of the bleach demand of the pulp.

12. The process of claim 11 in which the pulp concentration when treated with the hypochlorite is about 3 to 5%.

#### References Cited in the file of this patent

#### UNITED STATES PATENTS

2,676,885 Hamburg \_\_\_\_\_ Apr. 27, 1954

#### OTHER REFERENCES

Casey: "Pulp and Paper," vol. I, Interscience Publishers, 1952, page 273, 1st paragraph.